

May 3, 1960

J. SOTTYSIAK

2,935,405

STABILITY OF PHOTOGRAPHIC PAPER EMULSION COATINGS

Filed Aug. 25, 1955



FIG. 1



FIG. 2

INVENTOR  
JOSEPH SOTTYSIAK

BY *James W. Conley*  
*Edward P. Gilheany*  
ATTORNEY

1

2,935,405

## STABILITY OF PHOTOGRAPHIC PAPER EMULSION COATINGS

Joseph Sottysiak, Binghamton, N.Y., assignor to General Aniline & Film Corporation, New York, N.Y., a corporation of Delaware

Application August 25, 1955, Serial No. 530,615

6 Claims. (Cl. 96—110)

The present invention relates to photographic paper coatings and, specifically, to the improvement of gradation stability of photographic paper coatings prepared from chloro-bromide type photographic paper emulsions, while using strontium chloride in the precipitation of the silver halide.

It is well known in the photographic art that coated photographic emulsions are subject to change with age. This change may manifest itself as a loss in speed, maximum density and/or a general softening in gradation. This softening in gradation can be expressed as a loss in gamma ( $\gamma^-$ ) and a loss in maximum density when characteristic curves are plotted for the coated emulsion according to the well-known method of Hurter and Driffield (so-called H and D curve).

Photographic emulsions are generally coated on a paper base in various grades of contrast, i.e., soft, medium, hard and extra hard. The spacing between the gradations is so designated that photographic prints can be made by the usual methods of exposure to light from negatives of varying contrast. The photographic paper manufacturer attempts to stabilize these contrast spacings so they will maintain themselves throughout the life of the paper. In most cases, the commercial quality of a photographic paper is expected to continue for a period of up to two years, but considerable change occurs throughout the life of the paper. Various methods are used to obtain and maintain the spacing between contrasts. A common one is to coat the photographic emulsion at the highest limit of its contrast specification so that, upon aging and when ready for use, it will have leveled off at the designated gradation. This practice has many obvious deficiencies.

The other alternative is for the consumer to adjust processing conditions so as to compensate for shifts in paper quality. This is not satisfactory since he may have various contrasts of different coating ages. By my invention I intend to prepare a photographic paper emulsion which is considerably more stable toward change with aging by use of strontium chloride in the preparation of chloro-bromide type emulsions and while employing a critical quantity of strontium chloride during silver halide precipitation. The preparation of such emulsions and the emulsion so prepared constitute the purposes and objects of the present invention.

The literature pertaining to photographic emulsion making technique is quite meager. The use of certain chemicals during the precipitation of the silver halides in the carrier colloid gives photographic results totally unpredictable from a normal knowledge of their chemical properties.

Reference to the use of strontium chloride is given in Baker's "Photographic Emulsion Technique" where strontium and lithium chloride are used as a source of chloride ion in forming silver chloride in a collodion type chloride printing out paper. Reference in this same book is made to the fact that halides of barium, cadmium and other metals give warmer toned emulsions than do those of

2

potassium, sodium and ammonium. No other reference was found in the literature for the specific use of strontium chloride. As stated, I do not propose to use strontium chloride in the known relationship nor as a means of obtaining warmer tones, but as a gradation stabilizer.

I procure stabilization of gradation through the use of strontium chloride in combination with sodium chloride in the presence of other halides during the precipitation of silver halide in a carrier colloid such as gelatin to form a photographic paper emulsion. In the preparation of unwashed chloro-bromide emulsions, it is normal practice to use halide salts such as potassium bromide and sodium chloride and to form, by chemical interaction with silver nitrate in the presence of the carrier colloid such as gelatin, a silver bromide-silver chloride crystal complex. A small quantity, usually less than 10% of the bromide, of potassium iodide is added to give added sensitivity to the emulsion. Sodium chloride and potassium bromide are normally used as sources of halide ions because of their abundance, availability and favorable cost. Other metal halides can be used as sources of chloride ions. Strontium chloride in this invention is not used merely as a source of chloride ions, but as an adduct to the sodium chloride-potassium bromide combination. It is possible without strontium chloride to manufacture a suitable chloro-bromide emulsion but, surprisingly, with the addition of critical amounts of strontium chloride, a markedly superior product is obtained.

30 A chloro-bromide emulsion is prepared by interacting in the customary way in the presence of gelatin an aqueous solution of potassium bromide, sodium chloride and an amount of potassium iodide, not to exceed 10% of the potassium bromide, with silver nitrate so as not to completely precipitate all of the halide ions, but to leave a slight excess, not more than 15% of the total. This excess of halide in an unwashed emulsion is beneficial in stabilizing the emulsion against fog. At the proper temperature (50-75° C.) and with the appropriate silver nitrate addition, a photographic emulsion is obtained which is subsequently coated on a paper base. This emulsion has the characteristics of Figure 1 of the accompanying self-explanatory drawing which illustrates the invention by sensitometric curves prepared in the manner of Hurter and Driffield.

45 It is found that when the chloride salt concentration is changed so as to include the chlorides of strontium and sodium in a definite ratio of mol percentages, an emulsion is obtained which, when coated on a paper base, gives a product with the characteristics of Figure 2. F in each figure refers to the freshly coated paper exposed in a sensitometer to give a characteristic H and D curve. O, on the other hand, refers to the same coating exposed in a sensitometer after a four-day accelerated oven aging test effected at 140° F. (60° C.) and a relative humidity of 20-25%. This type of test treatment corresponds substantially to a normal natural aging of approximately one year. It will be observed that in Example I, there is considerable loss in gradation after aging, whereas in Example II, there is relatively little loss in gradation with aging.

50 It is necessary to operate within certain limits of halide salts to obtain the desired improvement. This range extends from a ratio of mol percent of (a) 12.0 of sodium chloride to one of strontium chloride to (b) 2.7 of sodium chloride to one of strontium chloride. Concentrations lower than the 12/1 ratio have little or no effect in improving gradational stability. Concentrations in a ratio higher than 2.7/1 give an emulsion with poor photographic properties. Thus, the emulsions are difficult to coat on a paper base and after aging, exhibit peculiar properties in normal photographic developer solutions.

The particular reasons for the improvement obtained have not been determined and are not easily explainable. Two theories present themselves but whether either is applicable is unknown. It is impossible to determine which of the halides present reacts with the silver nitrate. It is barely possible that the strontium chloride does not react or reacts only in part. This would mean that free strontium chloride is present in the emulsion, it being emphasized that the emulsion being a paper emulsion is unwashed.

It is noted, on the other hand, that in addition to the strontium chloride there is present potassium bromide, sodium chloride and potassium iodide. The possibility, therefore, exists that, upon reaction of the halides with silver nitrate, a peculiar heretofore unattainable crystal lattice is produced. However, regardless of the theory, the fact remains that by utilization of the various halides including strontium chloride and the particular ratio pointed out, new and unexpected results are obtained from the standpoint of gradational stability.

The following examples will serve to illustrate the invention but it is to be understood that the invention is not restricted thereto.

#### Example I

The following basic formula defines a composition with the lowest concentration of strontium chloride. The strontium chloride used is the normally available crystalline hexahydrate, i.e.,  $\text{SrCl}_2 \cdot 6\text{H}_2\text{O}$ . The mol percent is calculated on the actual  $\text{SrCl}_2$  present in the crystal.

|      |                    |     |        |    |
|------|--------------------|-----|--------|----|
| I.   | Potassium bromide  | g.  | 14.40  |    |
|      | Sodium chloride    | g.  | 8.40   |    |
|      | Strontium chloride | g.  | 3.20   |    |
|      | Potassium iodide   | g.  | 0.96   |    |
| II.  | Gelatin            | g.  | 98.20  | 35 |
|      | Water              | cc. | 690.00 |    |
| III. | Silver nitrate     | g.  | 36.00  |    |
|      | Water              | cc. | 360.00 |    |

The salts in I are dissolved in II at 40-60° C. and then III is added uniformly over a period of 20-30 minutes. The temperature is then raised to a level of 50-70° C. and the material digested for a period of 60 to 90 minutes. The emulsion is cooled and hardened. Prior to coating, it is remelted at 30-40° C., a sensitizing dye, stabilizers and other finals then added. The emulsion is then coated on a paper base.

#### Example II

The same basic formula was used as in Example I, excepting that the ratio of salts was as follows:

|    |                    |    |       |    |
|----|--------------------|----|-------|----|
| I. | Potassium bromide  | g. | 9.95  |    |
|    | Sodium chloride    | g. | 7.80  |    |
|    | Strontium chloride | g. | 12.70 | 55 |
|    | Potassium iodide   | g. | 0.96  |    |

#### Example III

The same basic formula was used as in Example I, excepting that the ratio of salts was as follows:

|    |                    |    |      |    |
|----|--------------------|----|------|----|
| I. | Potassium bromide  | g. | 9.95 |    |
|    | Sodium chloride    | g. | 7.85 |    |
|    | Strontium chloride | g. | 6.25 | 65 |
|    | Potassium iodide   | g. | 0.96 |    |

#### Example IV

An ordinary emulsion was prepared for use in comparison in those of Examples I, II and III with the following ratio of salts:

|    |                   |    |       |  |
|----|-------------------|----|-------|--|
| I. | Potassium bromide | g. | 9.95  |  |
|    | Sodium chloride   | g. | 12.50 |  |
|    | Potassium iodide  | g. | 0.96  |  |

5 The following table depicts the differences that exist on a mol percent basis with the aforesigned ratio of sodium chloride to strontium chloride:

| Example | Mol Percent |      |                 |     | Ratio,<br>$\text{NaCl}/\text{SrCl}_2$ |
|---------|-------------|------|-----------------|-----|---------------------------------------|
|         | KBr         | NaCl | $\text{SrCl}_2$ | KI  |                                       |
| 1.      | 43.0        | 50.7 | 4.2             | 2.1 | 12.0/1                                |
| 2.      | 31.0        | 49.0 | 17.8            | 2.2 | 2.75/1                                |
| 3.      | 33.7        | 54.2 | 9.7             | 2.4 | 5.6/1                                 |
| 4.      | 27.5        | 70.5 | —               | 2.0 | —                                     |

The emulsions in Examples I, II, III and IV were coated on a paper base and subsequently exposed in a sensitometer and developed so as to yield H and D curves. Samples of each of the coatings were aged in an oven for four days in the manner previously stated. These papers were exposed and processed under identical conditions.

20 The data extracted from these are compiled in the following table:

| Example | Gamma |      |        |
|---------|-------|------|--------|
|         | Fresh | Aged | Change |
| 1.      | 1.22  | 1.05 | -0.17  |
| 2.      | 1.80  | 1.70 | -0.10  |
| 3.      | 1.72  | 1.60 | -0.12  |
| 4.      | 1.75  | 1.50 | -0.25  |

An examination of the table shows that by my invention the changes which occur upon aging have been greatly minimized. Thus, the emulsions of Examples I, II and III have considerably better gradation stability than emulsions prepared according to usual practice.

I claim:

1. The process of producing an unwashed silver halide paper emulsion having improved gradation stability which comprises precipitating in a colloidal carrier therefore, a mixed silver halide by reacting silver nitrate with an aqueous solution of potassium bromide, sodium chloride, potassium iodide and strontium chloride in the presence of said colloidal carrier, the molar ratio of sodium chloride to strontium chloride being between 2.7 and 12 of the former to 1 of the latter.
2. The silver halide emulsion made by the process of claim 1.
3. The process as defined in claim 1 wherein the colloidal carrier is gelatin.
4. The process as defined in claim 1 wherein the sodium chloride and strontium chloride are present in the ratio of 8.4 parts by weight of the former to 3.2 parts by weight of the latter.
5. The silver halide emulsion made by the process of claim 3.
6. The silver halide emulsion made by the process of claim 4.

#### References Cited in the file of this patent

#### UNITED STATES PATENTS

2,401,051 Crouse et al. May 28, 1946

#### OTHER REFERENCES

Baker: Photographic Emulsion Technique (2nd edition), 1948, American Phot. Publishing Company, Boston, page 251. Copy in Division 67.